

May 26, 1970

D. R. DAVIS ET AL  
ELECTROSENSITIVE RECORDING ARTICLE  
AND METHOD OF MAKING THE SAME  
Filed Nov. 17, 1966

3,514,325



INVENTORS  
DALE R. DAVIS  
ROBERT W. KINGSTON

BY *A. C. Smith*  
ATTORNEY

3,514,325

## ELECTROSENSITIVE RECORDING ARTICLE AND METHOD OF MAKING THE SAME

Dale R. Davis, Mountain View, and Robert W. Kingston, Palo Alto, Calif., assignors to Hewlett-Packard Company, Palo Alto, Calif., a corporation of California  
Filed Nov. 17, 1966, Ser. No. 595,117  
Int. Cl. G03g 5/00; B44d 1/09

U.S. CL. 117—217

4 Claims

### ABSTRACT OF THE DISCLOSURE

An improved electro-sensitive recording medium and method of making the same provides a matrix of conductive particles in a cross-linked binder disposed on a conductive backing layer for improved resistance to surface abrasion by a surface-contacting writing electrode.

This invention relates to an improved electro-sensitive recording medium which responds to low voltage and low power writing signals, and to the method of making the same.

It is an object of the present invention to provide an improved electro-sensitive recording medium which provides contrasting marks or records in response to applied writing signals and which includes an electro-sensitive surface coating that resists abrasion and mechanical scraping at elevated recording temperatures by the recording electrode of recording apparatus.

It is another object of the present invention to provide a method for making an improved electro-sensitive recording medium.

In accordance with the method and means of the present invention, a thin layer of aluminum is deposited on

5 the thickness of the layer 13 as measured by its resistance per square should be within this range so that low voltage writing signals applied through narrow electrodes in contact with the surface of the recording medium may attain a sufficiently high current density to vaporize the aluminum in the contacted area, thereby exposing the backing material in the regions through which writing signal flowed. Lower resistances per square (i.e. thicker films) require considerably higher power to vaporize the aluminum layer in the contacted region and higher resistances per square (i.e. thinner films) require higher writing voltages (typically above 60 to 100 volts) to provide sufficient power to vaporize the aluminum layer. Thus, since the limits are not precise, the term "approximately" as used herein is intended to cover values of resistance per square which are as much as an order of magnitude away from the expressed limits but which are useful with higher power, high voltage writing signals. Thus if sufficiently transparent backing material 11 is used, a recording 15 on the present medium may serve as an optically-transmissive master in inexpensive reproduction or electro-optical reading of the recording medium.

20 The surface coating 17 is prepared according to one embodiment of the present invention as follows: 300 grams of conductive zinc oxide (New Jersey Zinc Co. grade 013 or 016) and 400 grams of tetrahydrofuran or methylethylketone are combined with 100 grams of an organic polymer such as Eponol 55B40 (Shell Chemical Co.) and 15 grams of polyisocyanate cross-linking 25 agent such as Mondur CB-60 (Mobay Chemical Co.). Other useful combinations of binder materials and cross-linking agents (some being aided by a catalyst) are described in Shell Chemical Co., Plastics and Resins Division, Technical Bulletin SC:64-51 and in the following table:

| Weight Ratio<br>of Zinc Oxide<br>to Binder | Binder                    | Cross-linker<br>Agent       | Percent cross-linker<br>(by weight<br>of Binder) | Catalyst                   | Percent<br>Cat. | Disper-<br>sion pot<br>life | Time             | Cure<br>Temp. (° F.) |
|--------------------------------------------|---------------------------|-----------------------------|--------------------------------------------------|----------------------------|-----------------|-----------------------------|------------------|----------------------|
| 4:1                                        | Eponol 55B40 <sup>1</sup> | Toluene diisocyan-<br>ate   | 50 mole percent                                  | None                       | 0               | 3 hrs                       | 7 days           | 72                   |
| 4:1                                        | do <sup>1</sup>           | do                          | 15 mole percent                                  | do                         | 0               | 4 hrs                       | do               | 72                   |
| 4:1                                        | do <sup>1</sup>           | Uformite <sup>2</sup> MX61  | 50 wt. percent                                   | do                         | 0               | 4 days                      | 24 hrs           | 200                  |
| 4:1                                        | do <sup>1</sup>           | do <sup>2</sup>             | 20 wt. percent                                   | do                         | 0               | 5 days                      | 24 hrs           | 200                  |
| 4:1                                        | do <sup>1</sup>           | do <sup>2</sup>             | 50 wt. percent                                   | p-Toluene sulfonic<br>acid | 1               | 3 days                      | 2 hrs            | 200                  |
| 4:1                                        | do <sup>1</sup>           | do <sup>2</sup>             | 20 wt. percent                                   | do                         | 1               | do                          | 2 hrs            | 200                  |
| 4:1                                        | do <sup>1</sup>           | Uformite <sup>2</sup> F-240 | 50 wt. percent                                   | None                       | 0               | 4 days                      | 24 hrs           | 250                  |
| 4:1                                        | do <sup>1</sup>           | CKM6254 <sup>3</sup>        | do                                               | do                         | 0               | do                          | 24 hrs           | 250                  |
| 4:1                                        | do <sup>1</sup>           | CYMEL <sup>4</sup> 245-8    | 10, 30, 50, wt. percent                          | p-Toluene sulfonic<br>acid | 1               | 2-3 days                    | 2 hrs            | 200                  |
| 4:1                                        | do <sup>1</sup>           | Mondur <sup>5</sup> CB-60   | 30, 60 wt. percent                               | None                       | 0               | 1, 2 days                   | 14 days<br>5 hrs | 72<br>175            |
| 3:1                                        | Vitel <sup>6</sup> PE200  | do <sup>5</sup>             | 10-50 wt. percent                                | do                         | 0               | 4 days                      | 3 wks            | 72                   |
| 3:1                                        | Butvar 76 <sup>7</sup>    | Uformite MX61               | 20 wt. percent                                   | do                         | 0               | 5 days                      | 24 hrs           | 200                  |

<sup>1</sup> Shell Chemical Co. <sup>2</sup> Rohm and Haas Co. <sup>3</sup> Union Carbide. <sup>4</sup> American Cyanamid. <sup>5</sup> Mobay Chemical Co. <sup>6</sup> Goodyear Rubber & Chemical Co. <sup>7</sup> Shawinigan Resins

backing material to form a conductive layer having a selected resistance per square unit area. A surface coating including zinc oxide in a conductive matrix which is bonded together in a cross-linked polymer binder is provided on the conductive layer to form a recording medium which produces contrasting marks in response to applied writing signals.

These and other objects of the invention will be apparent from a reading of this specification and an inspection of the accompanying drawing which shows electro-sensitive medium and recording apparatus according to the present invention.

In the drawing, there is shown an electro-sensitive recording medium 9 which may be prepared according to one embodiment of the present invention as follows: Aluminum is vacuum deposited or sputtered onto a suitable backing material 11 such as paper or plastic film using well known methods to form a thin conductive layer 13 having a resistance ranging from approximately one ohm to approximately one hundred ohms per square.

55 The ingredients selected for the surface coating are then finely ground and dispersed in a ball mill operating for several hours. The agitated mixture forms a dispersion which is then deposited on the aluminum layer 13 by suitable means such as reverse roll coating to a dry weight of about three pounds per one thousand square feet. The volatile fluids are then driven off in a drying 60 oven leaving the conductive particles and binder in the surface coating 17 about .5 mil thick on the aluminum layer 13. The coated medium is then baked typically at about 200° F. for four hours to produce the cross-linking reaction. The binder in the resulting conductive matrix 65 thus includes a three-dimensionally cross-linked polymer which provides a firm bond to the aluminum layer that does not exhibit viscous flow at elevated temperatures and hence that resists mechanical scraping and abrasion at the elevated temperatures encountered during recording. This has the advantage over conventional uncross-linked binders that the residue from the recorded regions 70 is a mere powdery substance which does not accumulate

around the recording electrode that contacts the surface of the recording medium. Heretofore, the conventional uncross-linked surface coatings of electro-sensitive recording media have exhibited substantial viscous flow at the elevated temperatures encountered during recording. There, the surface-contacting recording electrode scrapes off the softened binder which thus accumulates around the electrode as gummy globules that build up and interfere with the electrode contact.

Therefore, the improved electro-sensitive recording medium of the present invention is capable of producing a contrasting mark in region thereof through which electrical recording signal flows without producing substantial amounts of gummy rubble or objectionable residue that can build up around the surface-contacting recording electrode.

We claim:

1. An electro-sensitive recording medium which prior to recording contrasting records therein in response to applied electric writing signals, comprises:

a metal conductive layer on an insulating substrate; and  
a conductive coating matrix on the surface said conductive layer which is capable of directly producing a contrasting record at elevated temperatures associated with electrographic recording thereon, the coating matrix including conductive particles in a binder which is the reaction product of an organic polymer that is capable of forming molecular cross links and a molecular cross-linking agent that is capable of interacting with said organic polymer to form molecular cross links and which includes cross-linked molecules, whereby the cross-linked binder prevents substantial viscous flow of the binder at

elevated temperatures associated with electrographic recording thereon.

2. An electro-sensitive recording medium as in claim 1 wherein said conductive particles include particles of zinc oxide which are dispersed throughout said matrix.

3. The method of producing an electro-sensitive recording medium comprising the steps, performed prior to electro-sensitive recording thereon, of:

forming a surface coating on a conductive backing by depositing thereon a fluid dispersion comprising conductive particles, an organic binder that is capable of forming molecular cross links and a cross-linking agent that is capable of interacting with said organic binder to form molecular cross-links; and curing said surface coating to form molecular cross-links between said binder and agent.

4. The method of producing an electro-sensitive recording medium as in claim 3 comprising the preliminary step of: formulating the fluid dispersion from conductive particles for zinc oxide, an organic binder and a quantity of a cross-linking agent that is at least about ten percent by weight of said organic binder.

#### References Cited

##### UNITED STATES PATENTS

|           |         |        |         |
|-----------|---------|--------|---------|
| 3,207,601 | 9/1965  | Giaimo | 96—1.5  |
| 3,411,948 | 11/1968 | Reis   | 117—217 |

ALFRED L. LETVITT, Primary Examiner

C. K. WEIFFENBACH, Assistant Examiner

U.S. Cl. X.R.

96—1.8; 117—218